# EUROPEAN PATENT APPLICATION

(11) **EP 0 892 107 A1**
(43) Date of publication of application: **20.01.1999**
(21) Application number: 98305702.7
(22) Date of filing: 16.07.1998
(51) Int. Cl.: D21C 3/06, D21C 9/00

(54) **Preparation of mechanical wood pulps with reduced energy**

(30) Priority: 17.07.1997 US 52924 P
(71) Applicant: Donohue Inc., Montreal, Quebec H3A 3C6 (CA)
(72) Inventor: Barnet, Adrian J., St. Catharines, Ontario L2T 3B2 (CA)
(74) Representative: Smart, Peter John

(57) **Abstract**

A refiner mechanical pulp is produced employing a two stage refining operation with an interstage chemical treatment. Energy savings are achieved to substantiate the same overall pulp quality by employing a reduced application of energy in the first stage of refining having a maximum of about 0.75 MWh/odt of pulp.

## Description

### FIELD OF INVENTION

The present invention relates to the preparation of improved mechanical wood pulps with reduced refining energy useful in all papermaking applications.

### BACKGROUND OF THE INVENTION

The term "mechanical pulp" as used herein has its normal meaning in the art and refers to the product of disruption of a woody substance by mechanical action to yield a product consisting mainly of liberated and separated single woody fibres and their fragments and which is suitable for use in the manufacture of paper.

The term "fibre" as used herein also has its normal meaning in the art and refers to individual plant cells which make up the woody material and which, in softwoods, are known botanically as parenchyma cells and cracheids. These fibres inherently have diameters generally below 0.05 mm and in the case of wood species commonly used in pulp formation and paper making, such as, spruce, balsam, pine, aspen and poplar, considerably below 0.05 mm.

"Refiner pulps" are a class of mechanical pulps formed by passing particulated cellulosic fibrous material, usually wood chips through a small gap between two ribbed parallel plates rotating with respect to each other (known as a disc refiner). The procedure may be effected under pressure, typically about 1 to 2 atmospheres greater than atmospheric pressure, and at elevated temperature, such as, about 120°C, the product being known as "thermo mechanical pulp" (TMP). The refining process usually is effected in two or more stages. In a first stage, the fibres are separated and liberated and in a second stage, additional refining energy is supplied to increase the fibre flexibility and conformability, fibrillation and bonding. Usually about half the overall refining energy used in the refining process of about 2.0 to about 2.4 MWh/odt or higher is applied to the fibre-liberation stage.

In Canadian Patent No. 1,145,107, there is described a process for preparing a refiner pulp using a three-step operation, in which a conventional two-stage procedure for preparing a refiner mechanical pulp has an intermediate as inter-stage mild chemical treatment.

In this procedure, wood chips, which have not been softened by chemical action, are subject to mechanical action in a disc refiner to form a pulp consisting mainly of single wood fibres and fragments thereof, the pulp is subjected to chemical reaction with a soluble salt of sulfurous acid under certain specific elevated temperature and pressure conditions, and the chemically-treated pulp is subjected to mechanical action to refine the same and improve pulp quality to provide a refined pulp having a Canadian Standard Freeness of about 50 to about 700.

The interstage chemical treatment is effected at an elevated temperature of above about 110°c and under a superatmospheric pressure with an aqueous solution of a soluble salt of sulfurous acid, usually sodium sulfite, containing sufficient alkali to maintain a pH greater than about 3 during the treatment. The chemical treatment is effected at a temperature and for a time to enable reaction with the pulp to occur. The chemical treatment also is effected at a temperature and for a time insufficient to result in a treated pulp yield below about 85% by weight, preferably to maintain the yield above about 90% by weight.

Fiber-to-fiber bonding within a dry paper sheet formed from the pulp produced by the procedure of CP 1,145,107 is improved, thereby resulting in the desirable properties of increased tensile and burst strength and increase sheet density.

The energy levels employed in CP 1,145,107 to achieve a predetermined level of pulp quality, as determined by Canadian Standard Freeness (CSF), are discussed, as compared to the conventional refiner pulp formation. This effect is illustrated in Figure 1 of the Canadian patent.

### SUMMARY OF INVENTION

It has now been found that it is possible to improve the process of CP 1,145,107 by using a combination of low refining energy in the primary refining stage followed by effecting the interstage chemical treatment to specific sulfonation levels, to lower the overall energy consumption in the manufacture of a wood pulp of a given freeness below the levels required in CP 1,145,107.

Accordingly, in one aspect of the present invention, there is provided A method of preparing a refiner mechanical pulp, which comprises:
(a) subjecting wood chips which have not been softened by chemical action to mechanical action in disc refiner at a maximum applied energy of 0.75 MWh/odt to form a pulp consisting mainly of single wood fibers and fragments thereof,
(b) subjecting the pulp to chemical reaction with a soluble salt of sulfurous acid containing sufficient alkali to maintain a pH greater than about 3 during the treatment at an elevated temperature of above about 110°C and under a superatmospheric pressure at a temperature and for a time sufficient to form a chemically-created pulp having a degree of sulfonation from about 0.3 to about 2 wt% and insufficient to result in a chemically-treated pulp yield below about 85% by weight, and
(c) subjecting the chemically-treated pulp to mechanical action to refine the chemically-treated pulp and improve pulp quality to provide a refined pulp have a Canadian Standard Freeness of about 50 to about 700.

In the present invention, the maximum level of energy use in the primary stage of refining is about 0.75 MWh/odt (megawatt hours per oven dry tonne of pulp). This value compares with a minimum value of about 0.9 MWh/odt and a usual range of about 1.0 to about 1.2 MWh/odt as described in the aforementioned CP 1,145,107. Preferably, the energy level used is greater than about 0.4 MWh/odt. The first stage of refining is then followed by the interstage chemical treatment and subsequent refining steps.

While the interstage chemical treatment in CP 1,145,107 provided a lower overall energy requirement to a desired pulp freeness when compared with conventional refining to produce refiner mechanical pulp, it is possible, by operating at lower energy levels in the first stage in combination with specific levels of sulfonation, to provide a further decreased overall energy usage in preparing the refiner mechanical pulp.

In addition, by modifying the operating conditions of the interstage chemical treatment to provide higher yields but at the expense of lower pulp properties, further significant overall energy savings can be realized and still produce a pulp with wet web and other papermaking properties which are comparable or superior to those of thermomechanical pulp (TMP), although not as good as achievable using the conditions described in CP 1,145,107.

Accordingly, the present invention employs the mechanical refining with interstage chemical treatment procedure of Canadian Patent No. 1,145,107 but in a manner which surprisingly leads to an overall energy saving for the same final pulp freeness of refiner mechanical pulp as compared to pulp produced by procedures described in the Canadian Patent. In addition, the present invention enables there to be produced a pulp of paper-making properties similar to conventional thermomechanical pulp (TMP) of the same freeness at considerable energy savings in comparison to that required to produce TMP.

### BRIEF DESCRIPTION OF DRAWINGS

Figure 1 is a graphical illustration of the energy savings which are achievable following the procedure of the present invention;
Figure 2 is an illustration showing that the reduction in total specific energy applied in refining can be reduced as per the present invention without any major change in pulp properties;
Figure 3 is a graphical representation of the variation of wet web tensile strength with freeness at various levels of sulfonation, illustrating that the same wet web tensile strength can be achieved by combining both the degree of refining as measured by a drop in freeness and the degree of sulfonation;
Figure 4 is a graphical representation of the variation of bulk with freeness at various levels of sulfonation and illustrates that the same bulk can be reached by combining both the degree of refining as measured by a drop in freeness and the degree of sulfonation;
Figure 5 is a graphical representation of the variation of breaking length with freeness at various levels of sulfonation and illustrates that the same breaking length can be obtained by combining the degree of refining as measured by the drop in freeness and by the degree of sulfonation.
Figures 6, 7 and 8 are graphical representations of the variation in wet web tensile, bulk and breaking length respectively with refining time for the second stage of refining, illustrating the reduction in refining time achieved according to the invention, the level of energy reduction in the second stage of refining being proportional to the degree of sulfonation;
Figures 9 to 12 are graphical variations of the improvement in pulp properties which is obtained from the interstage sulfonation with a combination of softwood and hardwood pulps for a given level of sulfonation; and
Figure 13 is a graphical representation of the variation of refining time with freeness for a given degree of sulfonation, illustrating the energy saving realized by application of the invention with substantially less time being required to achieve the same freeness after cooking the pulp.

### GENERAL DESCRIPTION OF INVENTION

The process of the invention comprises three steps, namely (a) subjecting particulated cellulosic fibrous material to mechanical action in a disc refiner under specific condition of energy application to form a pulp consisting mainly of single fibres and fragments thereof, (b) chemical reaction of the pulp with a soluble salt of sulfurous acid under certain precise elevated temperature and pressure conditions as detailed below, to produce a desired level of sulfonation and (c) subjecting the chemically-treated pulp to mechanical action to refine the same and improve the pulp quality.

The cellulosic fibrous material species and refining conditions required to manufacture a usable mechanical pulp are well known to the art. For example, it is well known that most hardwoods cannot usefully be refined without a chemical pre-treatment to yield mechanical pulps with adequate strengths. Unlike the procedure described in CP 1,145,107, which is restricted to refiner pulps which are generated from softwoods, or other cellulosic fibrous material species which are recognized in the industry as being suitable for the preparation of refiner pulps. The procedure of the present invention enables hardwoods to be used to produce mechanical pulps of adequate pulp properties. For example, this benefit can be realized by co-refining a mixture of softwood and hardwood chips and cotreating the resulting chips. Typical results are seen in Figures 9 to 13. The invention is described further with particular reference to wood species.

The three individual steps comprising the process of the invention are discussed separately below:

### Step (a) Fibre Separation

A wood fibre consists essentially of a cell wall, whose outer surface is made up of cellulose-rich fibrillar layers known as the S₁ and S₂ layers. In wood, the space between the fibres, known as the middle lamellae, is filled with a lignin-rich material.

The process of the invention requires that, in the initial liberation of the fibre from the wood in a disc refiner, the fracture occurs mainly in the S₁ and S₂ layers, thus exposing the cellulose-rich fibrillar material which is the source of the fibrillation characteristics of a good mechanical pulp. Since this fibre morphology is established at the moment of fibre liberation, it is necessary that the process of fibre liberation proceed largely to completion. Therefore, the product of the initial mechanical fibre separation step of the process of the invention must consist mainly of single wood fibres, which inherently have average diameters less than 0.05 mm.

It is well known that, in thermomechanical pulping, if the refining temperature exceeds the thermal softening point of lignin, fibre separation occurs in the middle lamellae to yield a smooth fibre with a lignin-rich surface. This fibre is difficult or impossible to fibrillate by further refining and is generally unsuitable for use as a mechanical pulp. Hence the initial fibre separation step in this invention is effected at a temperature below the thermal softening point of lignin. The latter temperature is variable with the wood species, duration of heating and refining conditions but is generally below 150°C.

It has now surprisingly been found that the primary refining stage energy may be significantly decreased while maintaining the same level of interstage chemical treatment and subsequent refining energy while the freeness remains substantially unchanged.

In accordance with the present invention, the first stage of refining is affected at a maximum energy usage of about 0.75 MWh/odt, preferably greater than about 0.4 MWh/odt. The effect of the decreased energy use in the first stage of refining on final freeness and overall energy may be seen in Figure 1.

In generating the data seen in Figure 1, the primary stage refining energy was varied while the interstage chemical treatment was maintained at a temperature of about 160°C for about 40 minutes at a chemical application of about 8 wt% sodium sulfite at about pH 8.7 under a pressure of about 75 psig at a pulp consistency of about 30% to provide a degree of sulfonation of 1.7 to 1.8%. The second stage refining step which also included fibre rejected from screening stages was maintained at about 0.65 MWh/odt.

In Figure 1, there is shown the effect of reduction of primary specific energy (square boxes) on overall pulp freeness (diamond boxes). As may be seen, as the primary stage energy usage falls, the pulp freeness remains substantially unchanged, leading to a significant overall energy saving.

As is shown in Figure 2, the pulp properties as demonstrated by breaking length and tear remain essentially unchanged even though the specific energy applied in the first stage of refining was substantially reduced.

Primary stage refining is effected in the present invention at level below about 0.75 MWh/odt which is below any primary stage energy level contemplated in CP 1,145,107, wherein a minimum value of about 0.9 MWh/odt, usually about 1.0 to about 1.2 MWh/odt, is employed and leads to a significant overall energy requirement. This phenomenon of decreased primary stage refining while maintaining substantially the same freeness can be achieved through high intensity refining in the primary stage and/or by making a higher freeness pulp in the primary stage of refining. High intensity refining may be effected commercially in a number of ways, such as by increased refiner speed, increased throughput of the refiner or by manipulation of other refining parameters, such as consistency and plate pattern. A higher freeness pulp may be achieved by directly decreasing the energy applied in the first stage of refining.

### Step (b) Chemical Reaction

After the required physical form of the wood fibre is obtained in step (a), the chemical nature of the fibre is modified by reaction with an aqueous solution of a soluble salt of sulphurous acid, usually sodium sulphite, to sulfonate the fibers. The reaction is effected at temperatures above about 110°C under a superatmospheric pressure for a time sufficient to yield a chemically-treated mechanical wood pulp capable of forming a paper web having improved wet stretch and stress-strain properties and exhibiting rapid drainage, but for a time insufficient to cause substantial dissolution of lignin with consequent loss of yield and generation of polluting effluents. The exact nature of the chemical reactions involved in the chemical treatment effected in this invention are not fully understood, but involve sulfonation.

During the reaction, the pH of the solution drops and alkali is consumed. It is essential to the process of the present invention that sufficient alkali be present in the chemical charge to prevent a pH drop below 3 during treatment, otherwise there is a risk of damaging the fibres through hydrolytic action with consequent loss of strength. The exact amount of alkali required varies according to the acetyl content of the wood supply and cannot be specified exactly, but is rapidly established by experimentation.

The alkali requirement may be met entirely with sodium sulphite. However, since only half of the sodium of sodium sulphite is available for neutralization, it is usually more economical to meet part of the alkali requirements by additions of sodium hydroxide or sodium carbonate. The pH of the mixture, however, is preferably kept below about 12 because hemicelluloses are dissolved from wood fibre by higher pH's, with consequent loss in yield.

The chemical reaction is effected in accordance with the present invention under reaction condition necessary to achieve levels of sulfonation of the pulp from about 0.3 to about 2 wt%, preferably about 0.4 to about 1.8 wt%. Such levels of sulfonation may be achieved by utilizing selected combination of temperature, time and chemical concentration as the cooking conditions. As seen in Table 1 below, various levels of sulfonation may be achieved by varying these reaction conditions.

In an embodiment of the invention, the amount of sodium sulphite used in the chemical treatment is in the range of about 1% to about 15% by weight based on mechanical wood pulp resulting from step (a), preferably about 2 to about 10% by weight. The chemical charge preferably has a pH between about 7 to about 12, and contains sodium sulphite and sufficient alkali to maintain a pH greater than 3 throughout the reaction.

We have found that the maximum improvement, namely, maximum increase in wet stretch, maximum improvement in stress-strain, maximum increase in strength characteristics, and maximum decrease in refiner power requirements for the second stage (step (c) discussed below), is obtained from the process of the invention when the mechanical pulp from step (a) with added chemical is heated at about 160°C for 30 minutes. As with any other chemical reaction, the temperature can be lowered if the reaction time is increased. Below about 120°C, reaction time becomes impractically long, and below 110°C, the required reactions effectively cease. Similarly, the reaction temperature can be increased if the reaction time is shortened. The practical upper limit of temperature appears to be about 200°C with reaction times of 1 to 2 minutes. We prefer not to operate under these extreme conditions because the precise control of conditions and reaction times needed to achieve an optimum product and difficult to secure.

It is also possible to operate at shorter or longer than the optimum reaction times to produce a less than optimum but still useful result. If the reaction time is shorter than optimum, the improvements in wet stretch, stress-strain and strength properties and energy requirements are less than may be otherwise obtained by operating under optimum conditions. If the reaction time is too long, substantial dissolution of the lignin from the pulp, in the treating chemical occurs, with consequent loss of yield and formation of polluting effluent. While the process is still operable to produce property improvements under these conditions some of the advantages of wood economy and low pollution are lost and generally are avoided.

The chemical treatment is operable over a time-temperature range from about 110°C for about 12 hours to about 200°C for about 1 minute. It is understood that an increase in temperature must be accompanied by a concomittant decrease in reaction time.

Preferably, the temperature of the reaction varies from about 130° to about 160°C with reaction times from about 20 to 60 minutes. As noted above, such temperature/time profiles are employed in conjunction with chemical concentration to achieve the desired degree of sulfonation between about 0.3 to about 2 wt%, preferably about 0.4 to about 1.8 wt%.

### Step (c) Refining

In the third step of the process of the invention, the product of step (b) is subjected to further refining action, following the usual practice of the industry for subsequent refining of a mechanical wood pulp. Such subsequent refining may include a separate refining step. The results of this further refining action differ from those obtained with an ordinary mechanical wood pulp because the application of steps (a) and (b) in accordance with this invention places the pulp in the required physical and chemical configuration to utilize further refining energy efficiently and economically. It is well known that the quality of a mechanical wood pulp can be improved by increased refining, but at a cost of slower drainage and increased energy demand. The product of step (b) may be refined to equivalent quality with significantly less energy, while achieving a faster drainage, as compared to mechanical pulp from step (a) which has not been subjected to step (b).

In accordance with the invention, the same overall freeness and pulp quality of the three-stage process of CP 1,145,107 can be achieved herein at a reduced overall energy saving, as a result of the reduced application of energy in the first stage refining. In addition, if a lesser quality pulp comparable to conventional TMP is desired, such a product can be achieved with a considerably decreased overall energy usage as compared to the processes of TMP.

The amount of energy applied in step (c) may be varied according to the desired properties of the product and the intended end use. The degree of refining to which the pulp is subjected to usually controlled by the freeness of the finished pulp. For most applications, this freeness should fall within the range of about 50 to about 700 C.S.F. For example, boxboard stock is typically of higher freeness than magazine grade paper stock. For newsprint application, it is preferred to refine to a freeness in the range about 100 to about 400 C.S.F. in step (c).

### EXAMPLES

### Example 1

This Example illustrates the effect of interstage cooking condition on the degree of sulfonation.

Wood chips were subjected to primary stage refining at an energy level of 0.7 MWh/odt at various temperatures, times and sodium sulfite solution concentration at about pH 8.7 under a suitable superatmospheric pressure at a pulp consistency of about 35%. The results obtained are shown in Table 1 below.

Table 1 shows the impact of the variation in the time, temperature and amount of chemical added on the degree of sulfonation, illustrating that the severity of the cook may be manipulated to achieve a desired degree of sulfonation to the pulp.

### Example 2

This Example illustrates the effect of degree of sulfonation on wet web properties and the energy savings resulting therefrom.

The pulp samples obtained according to the procedure of Example 1 was formed into paper sheets and the variation of different wet web properties with degree of sulfonation was determined. These results are presented graphically in Figures 3 to 5.

Figure 3 shows that the same wet web tensile strength can be achieved by combining both the refining energy as measured by a drop in freeness and the degree of sulfonation. The reference TMP sample in these Figures is given by the legend "0% sulfonation".

Figure 4 shows that the same bulk value can be reached by combining both the refining energy as measured by a drop in freeness and the degree of sulfonation.

Figure 5 shows that the same breaking strength can be obtained by combining the refining energy as measured by the drop in freeness and by the degree of sulfonation.

In Figures 6, 7 and 8, the data shown in Figures 3, 4 and 5 respectively is re-presented in a form which shows the energy saving achieved by the present invention. As may be seen, the level of energy reduction achieved in the second stage of refining to achieve the same pulp freeness is proportional to the degree of sulfonation of the wood pulp in the interstage chemical treatment.

From the graphical representation of Figures 3 to 8, it can be seen that, at a degree of sulfonation of about 0.4% and higher, a pulp with superior properties to untreated TMP can be produced at about 300 ml higher CSF. Accordingly, when making a pulp with properties similar to that of the TMP, the overall energy saving for production of the final refiner pulp arises from three sources, the savings due to the chemical treatment, the savings due to matching TMP properties but at a higher freeness and the savings from minimum application of energy in the first stage of refining.

### Example 3

This Example illustrates the savings in energy achieved using a combination of hardwood and softwood to form the pulp.

The wet web properties of paper sheets were determined for a mixture of 50:50 hardwood/softwood pulp produced under the condition of sulfonation to provide 0.8 wt% sulfonation.

Figures 9 to 12 show the improvement in pulp properties due to the interstage treatment which can be obtained with a combination of hardwood/softwood pulps for a given level of sulfonation.

Figure 13 shows the decrease in overall energy saving which is achieved according to the invention. As seen therein, to achieve the same freeness level as the reference TMP, substantially less refining time and hence refining energy, is required after cooking the pulp.

### SUMMARY OF THE DISCLOSURE

In summary of this disclosure, the present invention provides novel procedure for producing pulps of paper-making properties the same as the superior to conventional TMP at an overall energy saving. Modifications are possible within the scope of the present invention.

**TABLE 1**

| Impact of Cooking Conditions on Degree of Sulfonation | | |
|---|---|---|
| COOK NO. | COOKING CONDITIONS TEMP(°C) /TIME (MIN)/CHEM (%) | DEGREE OF SULFONATION |
| 1 | 160/45/8 | 1.23% |
| 2 | 160/60/8 | 1.08% |
| 3 | 160/30/8 | 1.15% |
| 4 | 160/30/5 | 0.83% |
| 5 | 145/60/8 | 1.14% |
| 6 | 145/45/5 | 0.78% |
| 7 | 145/30/3 | 0.60% |
| 8 | 145/60/5 | 0.79% |
| 9 | 130/45/5 | 0.73% |
| 10 | 130/60/3 | 0.62% |
| 11 | 130/45/8 | 0.92% |
| 12 | 130/30/3 | 0.55% |
| 13 | 130/60/5 | 0.78% |
| 14 | 160/20/5 | 0.67% |
| 15 | 160/20/6 | 0.82% |
| 16 | 145/20/3 | 0.55% |
| 17 | 145/20/4 | 0.66% |
| 18 | 130/20/2 | 0.41% |
| 19 | 130/20/2 | 0.43% |

## Claims

1. A method of preparing a refiner mechanical pulp, characterized by:
(a) subjecting wood chips which have not been softened by chemical action to mechanical action in disc refiner at a maximum applied energy of about 0.75 MWh/odt to form a pulp consisting mainly of single wood fibers and fragments thereof,
(b) subjecting the pulp to chemical reaction with a soluble salt of sulfurous acid containing sufficient alkali to maintain a pH greater than 3 during the treatment at an elevated temperature of above 110°C and under a superatmospheric pressure at a temperature and for a time sufficient to form a chemically-treated pulp having a degree of sulfonation from 0.3 to 2 wt% and insufficient to result in a chemically-treated pulp yield below 85% by weight, and
(c) subjecting the chemically-created pulp to mechanical action to refine the chemically-treated pulp and improve pulp quality to provide a refined pulp have a Canadian Standard Freeness of 50 to 700.

2. The method claimed in claim 1 wherein said total applied energy during the step (a) is at least 0.4 MWh/odt up to said maximum value.

3. The method claimed in claims 1 or 2 wherein said soluble salt sulfurous acid is an aqueous medium sulfite solution and step (b) is effected at an applied chemical charge of 1 to 25% by weight of sodium sulfite based on pulp.

4. The method claimed in any one of claims 1 to 3 wherein said applied chemical charge is from 2 to 8 wt%.

5. The method claimed in any one of claims 1 to 4 wherein step (b) is effected at a temperature of 130° to 160°C for 20 to 60 minutes.

6. The method claimed in any one of claims 1 to 5 wherein said step (b) is effected under temperature/time/applied chemical conditions to provide a degree of sulfonation of 0.4 to 1.8 wt% at a pulp yield of at least 90% by weight.

7. The method claimed in any one of claims 1 to 6 wherein said wood chips include hardwood wood chips.

8. The method claimed in any one of claims 1 to 7 wherein said steps are carried out to produce a refined pulp having papermaking properties approximating those of conventional TMP.
